# EUROPEAN PATENT APPLICATION

(11) **EP 4 455 371 A2**
(43) Date of publication of application: **30.10.2024**
(21) Application number: 24163202.5
(22) Date of filing: 13.03.2024
(51) Int. Cl.: C25B 13/08, C25B 13/05, C25B 1/04, C25B 1/23, C25B 3/03, C25B 3/26, C25B 9/23, C25B 11/031, C25B 11/032, C25B 11/063, C25B 11/065, C25B 11/091

(54) **ELECTROLYSIS CELL AND ELECTROLYSIS DEVICE**

(30) Priority: 26.04.2023 JP 2023072196; 06.02.2024 JP 2024016578
(71) Applicant: Kabushiki Kaisha Toshiba, Tokyo 105-0023 (JP)
(72) Inventor: YONETSU, Maki, Tokyo, 105-0023 (JP); KIYOTA, Yasuhiro, Tokyo, 105-0023 (JP); KOFUJI, Yusuke, Tokyo, 105-0023 (JP); KITAGAWA, Ryota, Tokyo, 105-0023 (JP); MIKOSHIBA, Satoshi, Tokyo, 105-0023 (JP)
(74) Representative: Hoffmann Eitle

(57) **Abstract**

An electrolysis cell 20 includes: a cathode 31 to reduce a reducible gas; an anode 41 to oxidize an oxidizable substance in an electrolytic solution, the cathode 41 containing titanium; and a separator 50 separating the cathode 31 from the anode 41. The separator 50 includes a porous membrane. The porous membrane gives a pore size distribution defined by a graph having a horizontal axis and a vertical axis, the horizontal axis representing pore sizes of through holes of the porous membrane, the pore sizes being determined by using a porometer, the vertical axis representing a pore size flow distribution of pore volumes corresponding to the pore sizes, and the pore size distribution having a peak top in a range of not less than 0.01 µm nor more than 0.3 µm. The porous membrane has an ISO air permeance of not less than 0.8 µm/Pa·s nor more than 150 µm/Pa·s.

## Description

### FIELD

Arrangements relate to an electrolysis cell and an electrolysis device.

### BACKGROUND

In recent years, from both viewpoints of energy problems and environmental problems, it is desired not only to convert renewable energy such as sunlight into electric energy and use it but also to convert it into a storable and transportable state. In response to such a desire, research and development of Power to Chemicals technology of producing chemical substances using sunlight such as photosynthesis by plants are in progress. Such technology allows the renewable energy to be stored as storable fuel or the like, and promises to create value by producing chemical substances serving as industrial raw materials.

Known examples of devices which produce the chemical substances using the renewable energy such as sunlight, include a carbon dioxide electrolysis device which reduces carbon dioxide (CO₂) generated from facilities such as a power plant or an incinerator. The carbon dioxide electrolysis device includes a cathode (reduction electrode) which reduces carbon dioxide to produce a carbon compound such as carbon monoxide (CO) and an anode (oxidation electrode) which oxidizes water (H₂O) or a hydroxide ion (OH⁻). Such carbon dioxide electrolysis device preferably has a cell structure (electrolysis cell) formed by stacking the cathode and the anode with a separator such as an ion exchange membrane or a porous membrane therebetween, and the cell is directly supplied with carbon dioxide to a cathode catalyst layer of the cell to enable rapidly progress a reduction reaction of the carbon dioxide.

The electrolysis cell is to reduce crossover in the cell for improvement in its characteristics or the like. An example of the separator under review, which is disposed between the cathode and the anode, is formed using a porous membrane having a wide range of choices in its ion mobility and capable of achieving its high ion mobility. Unfortunately, the common porous membrane may form insufficient wet seals and thus prevent efficiently reduce of the crossover, depending on characteristics such as pore characteristics of the porous membrane. Thus, the cell is required to be improved in its characteristics by improving the porous membrane for the separator in its characteristics to improve wet sealing property of the separator.

### RELEVANT REFERENCES

### Patent Reference

Reference 1 : JPA 2022-145229
Reference 2 : JPA 2022-143970
Reference 3 : JPA 2022-143994

### BRIEF DESCRIPTION OF THE DRAWINGS

FIG. 1 is a diagram illustrating an electrolysis device of an arrangement.
FIG. 2 is a graph illustrating one example of a pore size distribution of through holes of a porous membrane determined by a porometer in the arrangement.
FIG. 3 is a graph illustrating one example of a pore size distribution of the porous membrane determined by a mercury intrusion method in the arrangement.

### DETAILED DESCRIPTION

An electrolysis cell of an arrangement includes: a cathode configured to be in contact with a reducible gas and to reduce the reducible gas; an anode configured to be in contact with an electrolytic solution containing an oxidizable substance and to oxidize the oxidizable substance, the anode containing titanium; and a separator separating the cathode from the anode. The separator includes a porous membrane. The porous membrane gives a first pore size distribution defined by a first graph having a first horizontal axis and a first vertical axis, the first horizontal axis representing first pore sizes of through holes of the porous membrane, the first pore sizes being determined by the porometer, the first vertical axis representing a pore size flow distribution of pore volumes corresponding to the first pore sizes, and the first pore size distribution having a first peak top in not less than 0.01 µm nor more than 0.3 µm. The porous membrane has an ISO air permeance of not less than 0.8 µm/Pa·s nor more than 150 µm/Pa·s.

Hereinafter, an electrolysis cell of an arrangement and an electrolysis device using it will be described with reference to the drawings. In each arrangement, substantially the same constituent parts are denoted by the same reference signs, and a description thereof may be partially omitted. The drawings are schematic, and the relation of the thicknesses of the parts and planar dimension, a thickness ratio among the parts, and so on may be different from actual ones. An example of applying the cell and the electrolysis device of the arrangement to an electrolysis cell and an electrolysis device of carbon dioxide (CO₂) will be mainly described in the following, but the cell and the electrolysis device of the arrangement are not limited to them. The cell and the electrolysis device of the arrangement may be applied to an electrolysis cell and an electrolysis device which electrolyzes nitrogen (N₂) to produce ammonia (NH₃), or the like, for example.

FIG. 1 is a diagram illustrating an electrolysis device of an arrangement. FIG. 1 illustrates a carbon dioxide electrolysis device 10 that includes an electrolysis cell 20. The cell 20 includes a cathode part 30, an anode part 40, and a separator 50 isolating them.

The cathode part 30 includes a reduction electrode (cathode) 31 having a metal catalyst layer, a cathode flow path 32, and a cathode current collector 33. The cathode flow path 32 is a gas flow path which supplies a carbon dioxide gas to the cathode 31 as a reducible gas (gas to be reduced), and is formed of a pit (groove) provided on a cathode flow path plate 34. The cathode 31 is disposed to enable being in contact with carbon dioxide flowing through the cathode flow path 32. The anode part 40 includes an anode (oxidation electrode) 41, an anode flow path 42, and an anode current collector 43. The anode flow path 42 is an electrolytic solution flow path which supplies an electrolytic solution as an anode solution to the anode 41, and is formed of a pit (groove) provided on an anode flow path plate 44. The electrolytic solution contains water (H₂O) or hydroxide ions (OH⁻) as an oxidizable substance (substance to be oxidized). The anode 41 is disposed to enable being in contact with the anode solution flowing through the anode flow path 42.

The carbon dioxide electrolysis device 10 includes a gas supply 60 which supplies carbon dioxide to the cell 20, and an electrolytic solution supply (supply system) 70 which supplies the anode solution to the cell 20. The gas supply 60 includes a CO₂ storage unit 61 such as a CO₂ gas cylinder and a CO₂ controlling unit 62 which regulates a flow rate of the CO₂ gas, and the CO₂ gas is supplied from the CO₂ storage unit 61 via a gas pipe 63 to the cathode flow path 32. The gas supply 60 may include a humidifying unit which humidifies the carbon dioxide gas. The carbon dioxide gas supplied to the cathode flow path 32 is not limited to a single gas of carbon dioxide, and may be a gas mainly composed of carbon dioxide (for example, a gas containing carbon dioxide of 90 vol% or more). To the cathode 31 of the cell 20 illustrated in FIG. 1, ions are supplied via the separator 50, and the carbon dioxide gas is supplied from the cathode flow path 32. A carbon dioxide reduction product is discharged mainly from the cathode flow path 32.

The electrolytic solution supply 70 includes an anode solution tank 71 and a pump 72, and the anode solution is supplied from the anode solution tank 71 via the pump 72 and an electrolytic solution pipe 73 to the anode flow path 42. The electrolytic solution supply 70 may have an anode solution-concentration measuring unit. The anode solution circulates through the anode flow path 42 and the electrolytic solution pipe 73. The cathode current collector 33 and the anode current collector 43 in the device 10 are connected to a power supply 80. The anode flow path plate 44 and the cathode flow path plate 34 is preferably formed using a material having low chemical reactivity and high conductivity. Examples of such material include a metal material such as titanium or SUS, carbon, or the like.

The cell 20 is commonly sandwiched by a pair of support plates, which are not illustrated, and further fastened by using bolts or the like. The power supply 80 connected to the cathode current collector 33 and the anode current collector 43 is not limited to an ordinary commercial power supply, a battery, or the like, and may be a power supply which converts renewable energy into electric energy and supplies it. Examples of such a power supply include a power supply which converts kinetic energy or potential energy such as wind power, water power, geothermal power or tidal power into electric energy, a power supply such as a solar cell with a photoelectric conversion element which converts light energy into electric energy, or the like, a power supply such as a fuel cell or a storage battery which converts chemical energy into electric energy, and a power supply such as a device which converts vibrational energy such as sound into electric energy. The use of renewable energy is also combined with effective use of carbon dioxide to be preferable in terms of the environment.

The cathode 31 is an electrode (reduction electrode) in which a reduction reaction of carbon dioxide (CO₂) as the reducible gas occurs to produce a carbon compound such as carbon monoxide (CO), methane (CH₄), ethane (C₂H₆), ethylene (C₂H₄), methanol (CH₃OH), ethanol (C₂H₅OH), or ethylene glycol (C₂H₆O₂). In the cathode 31, a side reaction in which hydrogen (H₂) is produced by the reduction reaction of water (H₂O) sometimes occurs simultaneously with the reduction reaction of carbon dioxide (CO₂). The cathode 31 has a first surface in contact with the separator 50, and a second surface facing the cathode flow path 32. The first surface of the cathode 31 is in contact with one surface of the separator 50.

The cathode flow path 32 which is a flow path of the gas containing CO₂ (hereinafter, also described as the CO₂ gas.) is formed of the pit (groove portion/recessed portion) provided in the cathode flow path plate 34. The cathode flow path plate 34 is provided with an inlet port and a discharge port of the gas of each of which illustration is omitted. Via the gas inlet port or the gas discharge port, the CO₂ gas is introduced from the gas supply 60. Moreover, via the gas inlet port or the gas discharge port, a reaction product gas containing CO, H₂, or the like is discharged, and the discharged gas is fed to a non-illustrated valuable material production part, or recovered to a product recovery part. The cathode flow path plate 34 and the cathode flow path 32 are provided to be in contact with the second surface of the cathode 31across the cathode 31 from the first surface of the cathode 31, the first surface being in contact with the separator 50.

The cathode 31 has a structure capable of moving ions and water between the separator 50 and the cathode flow path 32, for example, a porous structure such as a mesh material, a punching material, a porous member, or a metal fiber sintered member. The cathode 31 preferably includes a porous substrate containing carbon fibers, a gas diffusion layer and a catalyst layer, the gas diffusion layer and a catalyst layer being provided above the porous substrate in order, and a bulk density of the catalyst layer is preferably 0.1 g/cm³ or more and less than 0.6 g/cm³. A bulk density of the porous substrate with the catalyst layer and the gas diffusion layer, which is also referred to as an overall bulk density, is preferably not less than 0.1 g/cm³ nor more than 0.7 g/cm³. A catalyst material contained in the catalyst layer of the cathode 31 may have nanoparticles, a nanostructure, a nanowire, or the like for improving the reduction reaction. The nanostructure has nanoscale irregularities on a surface of the catalyst material or the like. The porous substrate is disposed to be adjacent to the cathode flow path 32, and the cathode catalyst layer is disposed to be adjacent to the separator 50. At least part of the cathode catalyst layer may enter into the gas diffusion layer. Thus, the cathode 31 has the porous structure. At least one of the porous substrate, the gas diffusion layer and the catalyst layer may have water repellency added by forming a surface covered with a fluorocarbon resin such as Teflon (registered trademark) as a water repellent agent. This addition is because movement of humidification water and the electrolytic solution, or the like causes a phenomenon in which the interior of a porous material is clogged with water (flooding), and has the possibility of decreasing characteristics of the cell 20. The bulk density may be a bulk density of the porous substrate with the water repellent agent. Further, the water repellent agent such as the fluorocarbon resin need not necessarily cover the surface of at least one member of the porous substrate, the gas diffusion layer, and the catalyst layer, or, for example, may be provided to be scattered inside the at least one of members (for example, between carbon fibers).

The cathode catalyst layer preferably has catalyst nanoparticles, a catalyst nanostructure, or the like. It is preferable that the porous substrate is composed of, for example, carbon paper, carbon cloth, or the like, and water repellent treatment is performed thereon. The cathode catalyst layer can receive ions to be supplied from the anode 41 via the separator 50. In the porous substrate, the CO₂ gas is supplied from and the product of the reduction reaction of the CO₂ gas is discharged from the cathode flow path 32. The reduction reaction of CO₂ occurs in a three-phase boundary of the cathode catalyst layer, and a gaseous product is discharged from the cathode flow path 32.

The cathode catalyst layer of the cathode 31 is preferably composed of the catalyst material (cathode catalyst material) capable of reducing CO₂ to produce the carbon compound, and capable of reducing an overvoltage in such a reaction. Examples of the cathode catalyst material include a metal material such as a metal such as gold (Au), silver (Ag), copper (Cu), platinum (Pt), palladium (Pd), nickel (Ni), cobalt (Co), iron (Fe), manganese (Mn), titanium (Ti), cadmium (Cd), zinc (Zn), indium (In), gallium (Ga), lead (Pb), or tin (Sn), or, an alloy or an intermetallic compound containing at least one of the above metals, a carbon material such as carbon (C), graphene, CNT (carbon nanotube), fullerene, or ketjen black, or a metal complex such as a Ru complex or a Re complex. The cathode catalyst layer may have at least one shape selected from a plate shape, a mesh shape, a wire shape, a particle shape, a porous shape, a thin film shape, and an island shape.

The anode 41 is the electrode (oxidation electrode) in which an oxidation reaction of water (H₂O) in the anode solution occurs to produce oxygen (O₂) and hydrogen ions (H⁺), or the oxidation reaction of hydroxide ions (OH⁻) produced in the cathode part 30 occurs to produce oxygen and water. The anode 41 is disposed between the separator 50 and the anode flow path 42 to be in contact with them. That is, the anode 41 has a first surface in contact with the separator 50, and a second surface facing the anode flow path 42. The first surface of the anode 41 is in close contact with the separator 50. The anode flow path plate 44 is connected to a solution inlet port and a solution outlet port (neither of them are illustrated), and the anode solution is introduced and discharged by the pump 72 via these solution inlet port and solution outlet port respectively. The anode solution can be circulated in the anode flow path 42 to be brought into contact with the anode 41. The anode current collector 43 is electrically connected to a surface of the anode flow path plate 44 defining the anode flow path 42, the surface being across the anode flow path plate 44 from a surface of the anode flow path 42, the surface facing on the anode 41.

When an aqueous solution of an electrolyte is used as the anode solution, the anode 41 is preferably mainly composed of a catalyst material (anode catalyst material) capable of oxidizing water (H₂O) to produce oxygen and hydrogen ions or oxidizing hydroxide ions (OH⁻) to produce water and oxygen, and capable of reducing an overvoltage in such a reaction. Examples of such catalyst material include a metal such as platinum (Pt), palladium (Pd), or nickel (Ni), an alloy or an intermetallic compound containing the above metals, a binary metal oxide such as a manganese oxide (Mn-O), an iridium oxide (Ir-O), a nickel oxide (Ni-O), a cobalt oxide (Co-O), an iron oxide (Fe-O), a tin oxide (Sn-O), an indium oxide (In-O), a ruthenium oxide (Ru-O), a lithium oxide (Li-O), or a lanthanum oxide (La-O), a ternary metal oxide such as Ni-Co-O, Ni-Fe-O, La-Co-O, Ni-La-O, or Sr-Fe-O, a quaternary metal oxide such as Pb-Ru-Ir-O or La-Sr-Co-O, or a metal complex such as a Ru complex or an Fe complex.

The anode 41 includes a base material (porous substrate) having a structure capable of moving the anode solution and ions between the separator 50 and the anode flow path 42, for example, a porous structure such as a mesh material, a punching material, or a porous sintered member. The porous substrate is composed of a titanium base material such as titanium or a titanium alloy having low reactivity. When an oxide is used as the anode catalyst material, a catalyst layer is preferably formed in a manner that the anode catalyst material is made to adhere to or stacked on a surface of the porous substrate composed of the metal material containing titanium. The anode catalyst material preferably has a shape of nanoparticles, a nanostructure, a nanowire, or the like for the purpose of increasing the oxidation reaction. The nanostructure is a structure having nanoscale irregularities on a surface of the catalyst material.

When the porous substrate of the anode 41 is composed of the material containing titanium, as described in detail later, titanium slightly is dissolved in operating the cell 20, and precipitates as a titanium oxide in a through hole of a porous membrane forming the separator 50. The titanium oxide precipitated in the through hole contributes to formation of wet seals in the separator 50, but too much dissolution of titanium has the possibility of causing hole clogging or the like in the porous substrate. Thus, in addition to titanium, the porous substrate preferably contains at least one element selected from the group consisting of tantalum (Ta), vanadium (V), molybdenum (Mo), zirconium (Zr), nickel (Ni), niobium (Nb), ruthenium (Ru), palladium (Pd), platinum (Pt), gold (Au), yttrium (Y), and iron (Fe). The presence of the at least one element reinforces the titanium oxide to cover an inner surface of the pore of the porous substrate to appropriately control the dissolution of the titanium. The at least one element is preferably each added in a range of not less than 0.1 mass% nor more than 5 mass% in the porous substrate containing the titanium.

Examples of the anode solution include an aqueous solution containing an optional electrolyte. Examples of the aqueous solution containing the electrolyte, include an aqueous solution containing phosphate ions (PO₄²⁻), borate ions (BO₃³⁻), sodium ions (Na⁺), potassium ions (K⁺), calcium ions (Ca²⁺), lithium ions (Li⁺), cesium ions (Cs⁺), magnesium ions (Mg²⁺), chloride ions (Cl⁻), hydrogen carbonate ions (HCO₃⁻), and carbonate ions (CO₃²⁻). A pH of the anode solution is not particularly limited, but preferably not less than 6 nor more than 10 in consideration of a use environment. Moreover, the anode solution is more preferably an alkaline solution containing HCO₃⁻, CO₃²⁻, LiHCO₃, NaHCO₃, KHCO₃, or the like.

The separator 50 can be composed of a material capable of moving ions between the anode 41 and the cathode 31 and capable of separating the anode part 40 and the cathode part 30, concretely, the porous membrane of an organic polymer material. The organic polymer material composing the porous membrane used for the separator 50 is not particularly limited, and examples of the organic polymer material include the fluorocarbon resin such as Teflon (registered trademark), a hydrocarbon polymer such as polyether, polysulfone, polyethylene, or polypropylene, cellulose, or the like.

The porous membrane of the separator 50 has through holes. The through holes of the porous membrane are filled with liquid such as the anode solution therein at the time of use of the cell 20, and the filling anode solution or the like allows movement of ions. That is, the porous membrane having the through hole functions as the separator 50 capable of moving ions between the anode 41 and the cathode 31. Moreover, filling the through holes of the porous membrane with the anode solution or the like in operating the cell 20 allows wet sealing between the anode 41 and the cathode 31, that is, inhibition of a movement of gases and liquid between the anode part 40 and the cathode part 30 and a reaction between the gases due to the movement (crossover).

To cause the porous membrane to have the function as the separator 50, that is, both the movability of ions and the inhibition of the crossover by using the wet seal by being filled with the anode solution or the like, the porous membrane applied to the separator 50 give a pore size distribution defined by a graph having a horizontal axis and a vertical axis, the horizontal axis representing pore sizes of the through holes, the pore sizes being determined by a porometer, the vertical axis representing pore size flow distribution of pore volumes corresponding to the determined pore sizes of the through holes (pore volumes of the through holes), the pore size distribution having a peak top in a range of not less than 0.01 µm nor more than 0.3 µm, and the porous membrane has an ISO air permeance of not less than 0.8 µm/Pa·s nor more than 150 µm/Pa·s. The ISO air permeance may be not less than 3 µm/Pa•s nor more than 150 µm/Pa•s, for example. The ISO air permeance may be not less than 0.8 µm/Pa•s nor more than 100 µm/Pa•s, for example. The ISO air permeance may be not less than 1.0 µm/Pa•s nor more than 100 µm/Pa•s, for example. The ISO air permeance may be not less than 1.0 µm/Pa•s nor more than 10 µm/Pa•s, for example. The determination of the ISO air permeance is based on JIS P 8117: 2009.

FIG. 2 illustrates one example of the pore size distribution determined by the porometer. A peak top of less than 0.01 µm in such the pore size distribution or an ISO air permeance of less than 0.8 µm/Pa•s makes the through hole likely to be clogged with a member peeled from the members during the operation, a re-precipitated substance of a dissolved member, or the like, which makes the function of the separator 50 and the characteristics of the cell 20 using it likely to decrease. An ISO air permeance of 1.0 µm/Pa•s or more makes the hole less likely to be completely filled in with aggregated particles of the catalyst separated from the cathode 31 even though the electrolytic solution or water vapor flows into the porous membrane with condensed water, which makes it difficult to inhibit the movement of ions in a membrane thickness direction, for example. An ISO air permeance of 3 µm/Pa•s or more makes the through holes less likely to be clogged with the anode solution therein, which allows prevention of a decrease in the function of the separator 50 and the characteristics of the cell 20 using it. An ISO air permeance of 10 µm/Pa•s or less increases an existing amount of the solution in the membrane, which allows a decrease in membrane resistance, for example. A peak top of more than 0.3 µm in the pore size distribution or an ISO air permeance of more than 150 µm/Pa•s makes the anode solution filling the through hole therein likely to escape, which decreases a wet sealing property between the anode 41 and the cathode 31, or decreases formability itself of the wet seal. These also make the characteristics of the cell 20 likely to decrease. An ISO air permeance of 100 µm/Pa•s or less allows retention of liquid in the membrane, which allows the formation of the wet seal during the operation, and the inhibition of the crossover of the gas, for example.

FIG. 3 illustrates one example of a pore size distribution determined by a mercury intrusion method. The porous membrane applied to the separator 50 preferably gives a pore size distribution defined by a graph having a horizontal axis and a vertical axis, the horizontal axis representing pore sizes of pores of the porous membrane, the pore size being determined by the mercury intrusion method, the vertical axis representing differential pore volumes corresponding to the determined pore sizes (differential pore volumes of the pores), the pore size distribution having a peak top in a range of not less than 0.05 µm nor more than 1 µm. Pore sizes of clogged holes (non-through holes) in a surface of the porous membrane is determined by the mercury intrusion method. A peak top of more than 1 µm in the pore size distribution determined by such a mercury intrusion method prevents effective formation of the wet seal, and causes the crossover of the gases and the liquid between the anode 41 and the cathode 31, which makes performance likely to decrease.

The peak top in the pore size distribution of the porous membrane determined by the porometer is more preferably not less than 0.01 µm nor more than 0.2 µm. The peak top in the pore size distribution of the porous membrane determined by the mercury intrusion method is more preferably not less than 0.05 µm nor more than 0.8 µm.

The pore size distribution of the porous membrane determined by the porometer, can be determined using, for example, POROLUX 1000 manufactured by Porometer N.V. or a measuring device equivalent to POROLUX 1000. The pore size distribution of the porous membrane by using the mercury intrusion method is determined using, for example, AutoPore V9610 manufactured by Micromeritics Instrument Corporation or a measuring device equivalent to V9610. The ISO air permeance of the porous membrane is determined using, for example, G-B3C manufactured by Toyo Seiki Seisaku-sho Ltd. or a measuring device equivalent to G-B3C.

When the porous membrane having the through hole is applied to the separator 50, for the use of the metal material containing titanium for the porous substrate of the anode 41, the titanium oxide having hydrophilicity precipitates in the interior and on a surface of the through hole at the time of operation of the cell 20, which allows an increase in formability of the wet seal through the hydrophilicity of the titanium oxide. In the titanium oxide is precipitated, the peak top in the range of not less than 0.01 µm nor more than 0.3 µm in the pore size distribution of the porous membrane determined by the porometer and the ISO air permeance of the porous membrane of not less than 0.8 µm/Pa•s nor more than 150 µm/Pa•s allow titanium oxide to suitably precipitate in the interior and on the surface of the through hole.

When the peak top in the pore size distribution of the through holes of the porous membrane determined by the porometer or the ISO air permeance is too small, an insufficient precipitation amount of the titanium oxide prevents the wet sealing property from sufficiently increasing. When the peak top in the pore size distribution of the through holes of the porous membrane determined by the porometer or the ISO air permeance is too large, an excessive precipitation amount of the titanium oxide has the possibility of causing a decrease in ion conductivity, or the like due to the clogging of the through hole, or the like. That is, applying the porous membrane in which the peak top in the pore size distribution of the through holes determined by the porometer and the ISO air permeance have suitable values allows the titanium oxide with a suitable amount to be precipitated in the through holes of the porous membrane. Consequently, the formability and safety of the wet seal can be sufficiently enhanced.

The amount of the titanium oxide to be formed in the through holes of the porous membrane, is preferably controlled so that titanium is contained in at least one pore of the porous membrane when the cell 20 is operated at a current density of 200 mA/cm² or more for 1000 hours or longer, for example. Moreover, an amount of the titanium in pores of the porous membrane may be defined by a mass ratio of a mass of any titanium compounds including titanium oxide to a mass of carbon in the porous membrane composed of the organic polymer material, and the mass ratio of the mass of any titanium compounds in the at least one pores is preferably 0.0001 or more when the mass of carbon in the porous membrane is relatively assumed to 1. The mass ratio is preferably 1 or less. These can improve a property such as the repeatability of the wet sealing property caused by the titanium oxide.

When the separator 50, which has the porous membrane with the titanium oxide precipitated in the at least one through hole, is divided in half thickness into a first porous part adjacent to the cathode 31 and a second porous part adjacent to the anode 41, a mass of any titanium compounds contained in the anode porous part is preferably larger than a mass of any titanium compounds contained in the cathode porous part. This allows the pores in the porous membrane to be effectively filled with the electrolytic solution having a sufficient concentration and flowing to the anode 41, resulting in continuing stable characteristics.

Such a porous membrane composed of the organic polymer material and used for the separator 50 as described above can be manufactured as follows, for example. Example methods of manufacturing of an organic polymer porous membrane, include various methods such as a phase separation method, a melt quenching method, an extraction method, a chemical treatment method, a stretching method, an irradiation etching method, a melting method, a foaming method, a compounding method, and fiber hollowing, and the example methods are not particularly limited. Among them, there can be used a method, referred to as a nonsolvent-induced phase separation (NIPS) method, in which bringing a homogeneous membrane-forming raw material solution obtained by dissolving an organic polymer in a solvent into contact with a coagulating solution containing a nonsolvent causes a concentration gradient between the solvent in the membrane-forming raw material solution and the nonsolvent in a coagulation bath, and the nonsolvent substitutes for the solvent in the membrane-forming raw material solution by using the concentration gradient as driving force to thereby promote a phase separation phenomenon, or a method of manufacturing using a thermally induced phase separation phenomenon in which cooling a polymer solution dissolved at high temperatures induces phase separation to increase pores, or there can be selected a method in which for such a material likely to become fibers as the fluorocarbon resin, fine pores are provided in the membrane by applying shear force, or the like. Further, combining these methods allows a predetermined porous structure to be obtained, and an inorganic substance may be compounded with the membrane, or coating for controlling the hydrophilicity may be performed on a surface. Further, a plurality of the membranes may be superposed.

The carbon dioxide gas supplied to the cathode flow path 32 may be supplied in a dry state, but is more preferably humidified. When the porous membrane of the organic polymer material is applied to the separator 50, using the carbon dioxide gas in the humidified state facilitates the formation of the wet seal in the porous membrane of the organic polymer material. The wet seal prevents the crossover between the anode part 40 and the cathode part 30 as described above. To humidify the carbon dioxide gas, the gas supply 60 may include the humidifying unit which humidifies the carbon dioxide gas flowing through the gas pipe 63. The humidifying unit (humidifying device) includes, for example, a humidification water tank, and is configured to humidify the carbon dioxide gas by vaporizing humidification water using an ultrasonic oscillator or the like. Further, the carbon dioxide gas may be humidified by being bubbled in the humidification water tank and passed therethrough.

Next, an operation of the device 10 illustrated in FIG. 1 will be described. Here, a case of producing carbon monoxide (CO) as the carbon compound is mainly described. However, the carbon compound as the reduction product of carbon dioxide is not limited to carbon monoxide, and may be methane (CH₄), ethane (C₂H₆), ethylene (C₂H₄), methanol (CH₃OH), ethanol (C₂H₅OH), ethylene glycol (C₂H₆O₂), or the like, and moreover, carbon monoxide which is the reduction product may be further reduced to produce the organic compounds.

First, the reaction process when water (H₂O) is oxidized mainly to produce hydrogen ions (H⁺) is described. When current is supplied from the power supply 80 between the anode 41 and the cathode 31, an oxidation reaction of water (H₂O) occurs in the anode 41 with which the anode solution is brought into contact. Concretely, as presented in the following formula (1), H₂O contained in the anode solution is oxidized, and oxygen (O₂) and hydrogen ions (H⁺) are produced.

2H₂O → 4H⁺ + O₂ + 4e⁻ ... (1)

H⁺ produced in the anode moves in the electrolytic solution existing in the anode 41 and the separator 50, and reaches the vicinity of the cathode 31. The reduction reaction of carbon dioxide (CO₂) occurs by using electrons (e⁻) based on the current supplied from the power supply 80 to the cathode 31 and H⁺ moved to the vicinity of the cathode 31. Concretely, as presented in the following formula (2), CO₂ supplied from the cathode flow path 32 to the cathode 31 is reduced to produce CO. Further, as presented in the following formula (3), hydrogen ions (H⁺) receive electrons, thereby producing hydrogen. At this time, hydrogen may be produced simultaneously with the production of carbon monoxide.

2CO₂ + 4H⁺ + 4e⁻ → 2CO + 2H₂O ... (2)

2H⁺ + 2e⁻ → H₂ ... (3)

Next, the reaction process when carbon dioxide (CO₂) is reduced mainly to produce hydroxide ions (OH⁻) is described. When current is supplied from the power supply 80 between the anode 41 and the cathode 31, in the vicinity of the cathode 31, as presented in the following formula (4), water (H₂O) and carbon dioxide (CO₂) are reduced to produce carbon monoxide (CO) and hydroxide ions (OH⁻). Further, as presented in the following formula (5), water receives electrons, thereby producing hydrogen. At this time, hydrogen may be produced simultaneously with the production of carbon monoxide. The hydroxide ions (OH⁻) produced by these reactions diffuse in the vicinity of the anode 41, and as presented in the following formula (6), the hydroxide ions (OH⁻) are oxidized to produce oxygen (O₂).

2CO₂ + 2H₂O + 4e⁻ → 2CO + 4OH⁻ ... (4)

2H₂O + 2e⁻ → H₂ + 2OH⁻ ... (5)

4OH⁻ → 2H₂O + O₂ +4e⁻ ... (6)

The carbon dioxide electrolysis device 10 of the arrangement as described above is not only specialized in only the reduction of carbon dioxide, but also, for example, can produce carbon monoxide and hydrogen at 1:2, and produce a carbon dioxide reduction product and hydrogen at an optional ratio at which methanol is produced in a chemical reaction thereafter, or the like. Hydrogen is a material which is inexpensive and easy to obtain through the electrolysis of water and from fossil fuel, and thus a ratio of hydrogen is not required to be large. A ratio of carbon monoxide to hydrogen is at least 1 or more, and desirably 1.5 or more from these viewpoints, which is preferable from economical and environmental viewpoints.

As described above, the device 10 of the arrangement controls the pore size of the through hole and the ISO air permeance of the porous membrane used as the separator 50 to suitable values allows improvement in the wet sealing property of the separator 50 in operating the cell 20. This allows, in operating of the cell 20, the inhibition of the movement of the gases and the liquid between the anode part 40 and the cathode part 30 and the reaction between the gases due to the movement, that is, the occurrence of the crossover. Consequently, the device 10 can be stably operated over a long period of time.

### Examples

Next, examples and evaluation results thereof will be described.

### (Examples 1 to 13, Comparative examples 1 to 3)

a composing material of a cathode catalyst layer, catalytic particles in which Au nanoparticles (metal catalyst) each having an average diameter of 2 nm were supported on carbon particles, and a Nafion solution (trade name, manufactured by Du Pont de Nemours, Inc.) as an ion-conductive material (ion-exchange resin) were prepared. The composing material, pure water, and isopropanol were mixed at predetermined ratios to prepare catalyst coating solutions.

Sheets of carbon paper with a diffusion layer having a microporous layer were each prepared as an electrode base material. A spray nozzle was filled with the catalyst coating solutions, which were sprayed on the sheets of carbon paper disposed on a heated hot plate, and spray coating was performed to be in such conditions as presented in Table 1. A mass of the metal catalyst per unit area of the catalyst layer was set to 0.15 mg/cm². These were cut into a size of 4 cm × 4 cm to serve as cathodes (each electrode area: 16 cm²). The detailed conditions are as presented in Table 1.

As anodes, an electrode in which a titanium nonwoven fabric was coated thereon with IrO₂ nanoparticles serving as a catalyst was used as a base, and elements presented in Table 1 were each added thereto. The element addition to the titanium nonwoven fabrics formed thin films of the elements on the titanium nonwoven fabrics, and the thin films were alloyed by heat treatment. The IrO₂/(the alloy layers of the additive elements and titanium/formation as necessary)/titanium nonwoven fabrics were cut into 4 × 4 cm to serve as the anodes (each electrode area: 16 cm²).

As separators, membranes presented in Table 1 were used. In Table 1, regarding peak tops in pore size distributions of through holes determined by using a porometer and peak tops in pore size distributions determined by mercury intrusion, values were read from graphs as FIG. 2 and FIG. 3 illustrated a case of the separator of Example 1. The separators in Examples 1 to 13 were porous membranes using organic polymer materials presented in Table 1, and the pore size distributions were prepared by controlling the conditions at the time of previously-described production. The measurements of the pore size distributions of the separators using the mercury intrusion method and the porometer, are performed in consideration of only a peak top in a range of 10 µm or less, and in no consideration of a peak in a range of more than 10 µm. This is because the peak in the range of more than 10 µm can be, for example, a peak caused by detecting a space between the membrane and the membrane as a pore.

Next, an electrolysis cell was fabricated. A cathode current collector, a cathode gas flow path, the cathode, the separator, the anode, an anode solution flow path, and an anode current collector were stacked in that order from the top, and sandwiched by support plates, and further fastened by bolts to fabricate the cell. The anode current collector and the cathode current collector were connected to an external power supply, an electrolytic solution was made to flow through the anode solution flow path, and a carbon dioxide gas was made to flow through the cathode gas flow path, resulting in fabricating a carbon dioxide electrolysis device.

**[Table 1]**

| | Anode | Separator | | | | | Cathode | | | | | |
|---|---|---|---|---|---|---|---|---|---|---|---|---|
| | Contained element | Membrane | | Pore size (1) | Pore size (2) | ISO air permeability | Catalyst layer | Overall | Mass ratio (3) | Pore size (1) | Pore size (2) | ISO air permeability |
| | | Membrane structure | Membrane material | Peak top position [µm] | Peak top position [µm] | [µm/Pa·s] | bulk density [g/cm³] | bulk density [g/cm³] | | Peak top position [µm] | Peak top position [µm] | [µm/Pa·s] |
| Example 1 | Ti,Ir | Porous membrane 1 | Polysulfone | 0.1 | 0.1 | 40 | 0.2 | 0.19 | 0.3 | 0.5 | 5 | 20 |
| Example 2 | Ti,Ir,Ta | Porous membrane 2 | Polyethersulfone | 0.14 | 0.15 | 55 | 0.22 | 0.2 | 0.4 | 0.8 | 30 | 25 |
| Example 3 | Ti,Ir,Y | Porous membrane 3 | Teflon | 0.15 | 0.15 | 56 | 0.18 | 0.19 | 0.2 | 0.45 | 4 | 15 |
| Example 4 | Ti,Ir,Fe | Porous membrane 4 | Polyethersulfone | 0.12 | 0.11 | 48 | 0.35 | 0.25 | 0.3 | 0.7 | 18 | 23 |
| Example 5 | Ti,lr,Ru | Porous membrane 5 | Polysulfone | 0.17 | 0.17 | 60 | 0.15 | 0.17 | 0.35 | 0.2 | 8 | 5 |
| Example 6 | Ti,Ir,Ta | Porous membrane 6 | Teflon | 0.08 | 0.08 | 30 | 0.25 | 0.19 | 0.3 | 0.4 | 20 | 17 |
| Example 7 | Ti,Ir,Zr | Porous membrane 7 | Polysulfone | 0.19 | 0.21 | 80 | 0.3 | 0.25 | 0.5 | 0.5 | 15 | 30 |
| Example 8 | Ti,Ir,Ta | Porous membrane 8 | Polyethersulfone | 0.2 | 0.5 | 100 | 0.1 | 0.19 | 0.1 | 1 | 50 | 50 |
| Example 9 | Ti,Ir,Ta | Porous membrane 9 | Teflon | 0.25 | 1.2 | 130 | 0.5 | 0.7 | 0.14 | 1.5 | 40 | 66 |
| Example 10 | Ti,Ir,Ta | Porous membrane 11 | Polyethersulfone | 0.15 | 0.15 | 2.5 | 0.23 | 0.21 | 0.35 | 0.90 | 50 | 25 |
| Example 11 | Ti,Ir,Ta | Porous membrane 12 | Teflon | 0.11 | 0.12 | 1.2 | 0.22 | 0.22 | 0.40 | 0.82 | 32 | 20 |
| Example 12 | Ti,Ir,Ta | Porous membrane 13 | Polyvinylidene fluoride | 0.17 | 0.18 | 3.8 | 0.25 | 0.24 | 0.33 | 0.68 | 58 | 26 |
| Example 13 | Ti,Ir,Ta | Porous membrane 14 | Polyethersulfone | 0.20 | 0.19 | 5.0 | 0.21 | 0.22 | 0.35 | 0.77 | 49 | 23 |
| Comparative example 1 | Ti,Ir | Anion exchange membrane | Polyarylpiperidiniu m | Outside measurement range | Outside measurement range | 0 | 0.6 | 0.75 | 0.7 | 0.05 | 1.5 | 0.1 |
| Comparative example 2 | Ti,Ir | Cation exchange membrane | Perfluorocarbon | Outside measurement range | Outside measurement range | 0 | 0.7 | 0.75 | 0.8 | 0.07 | 1.8 | 0.2 |
| Comparative example 3 | Ti, Ir | Porous membrane 10 | Teflon | 0.8 | 1 | 300 | 0.8 | 0.5 | 0.8 | 0.08 | 1.9 | 0.4 |

| | | | | | | | | | | | | |
|---|---|---|---|---|---|---|---|---|---|---|---|---|
| (1) Measured by porometer, (2) Measured by mercury intrusion method, (3) Mass of ion conductive substance/mass of metal catalyst | | | | | | | | | | | | |

Next, the electrolysis devices in Examples 1 to 13 and Comparative examples 1 to 3 were each operated under the conditions indicated below. The humidified carbon dioxide gas was supplied to the cathode gas flow path in a predetermined amount, and the electrolytic solution (an aqueous sodium hydrogen carbonate solution with a concentration of 0.1 M) was supplied to the anode solution flow path. A constant current of 200 mA/cm² was continuously applied between the anode and the cathode to perform an operation for 1000 hours. The separators after the operation for 1000 hours were taken out, and containing elements were analyzed using an ICP analysis and an infrared absorption method through high-frequency induction heating furnace combustion of the dissolved solutions. Table 2 presents analysis results, and retention rates of Faraday efficiency of CO after the operation for 1000 hours.

**[Table 2]**

| | Mass of Ti compound in separator to mass of carbon | Retention rate of CO Faraday efficiency after 1000-H operation [%] |
|---|---|---|
| Example 1 | 0.0003 | 99.8 |
| Example 2 | 0.0002 | 99.9 |
| Example 3 | 0.00015 | 99.6 |
| Example 4 | 0.0002 | 97.6 |
| Example 5 | 0.001 | 99.5 |
| Example 6 | 0.01 | 98.6 |
| Example 7 | 0.00018 | 95.1 |
| Example 8 | 0.00014 | 93 |
| Example 9 | 0.0001 | 90.1 |
| Example 10 | 0.0002 | 99.9 |
| Example 11 | 0.00015 | 99.7 |
| Example 12 | 0.00022 | 99.8 |
| Example 13 | 0.00031 | 99.8 |
| Comparative example 1 | 0 | Impossibility of 1000-H operation |
| Comparative example 2 | 0 | Impossibility of 1000-H operation |
| Comparative example 3 | 0.00005 | 10 |

As presented in Table 2, for the use of the separators in ranges of Examples, in any sample, as a mass of a titanium compound in the separator after the operation for 1000 hours, a ratio of a mass of the titanium compound to a mass of carbon of the separator was 0.0001 or more, and the retention rate of the CO Faraday efficiency after 1000 hours was also high to be 90% or more. On the other hand, for the use of membranes having no porosity and a porous membrane with a pore size distribution range of the membrane outside as in Comparative examples, cell characteristics decreased before the operation for 1000 hours, and retention rates of the CO Faraday efficiency were also low, or the operation for 1000 hours failed to continue.

The configurations of the arrangements are applicable in combination with each other, and parts thereof are also replaceable. While certain arrangements of the present invention have been described above, these arrangements have been presented by way of example only, and are not intended to limit the scope of the invention. Indeed the novel arrangements described herein may be embodied in a variety of other forms; furthermore, various omissions, substitutions, and changes in the form of the arrangements described herein may be made without departing from the spirit of the inventions. The accompanying claims and their equivalents are intended to cover such forms or modifications as would fall within the scope and spirit of the inventions.

The arrangements can be summarized into the following clauses, for example.

### (Clause 1)

An electrolysis cell comprising:
a cathode configured to be in contact with a reducible gas and to reduce the reducible gas;
an anode configured to be in contact with an electrolytic solution containing an oxidizable substance and to oxidize the oxidizable substance, the anode containing titanium; and
a separator separating the cathode from the anode, wherein:
   the separator includes a porous membrane;
   the porous membrane gives a first pore size distribution defined by a first graph having a first horizontal axis and a first vertical axis, the first horizontal axis representing first pore sizes of through holes of the porous membrane, the first pore sizes being determined by the porometer, the first vertical axis representing a pore size flow distribution of pore volumes corresponding to the first pore sizes, and the first pore size distribution having a first peak top in not less than 0.01 µm nor more than 0.3 µm; and
   the porous membrane has an ISO air permeance of not less than 0.8 µm/Pa·s nor more than 150 µm/Pa·s.

### (Clause 2)

The cell according to clause 1, wherein
the porous membrane gives a second pore size distribution defined by a second graph having a second horizontal axis and a second vertical axis, the second horizontal axis representing second pore sizes of the porous membrane, the second pore sizes being determined by a mercury intrusion method, the second vertical axis representing log differential pore volumes corresponding to the second pore sizes, and the second pore size distribution having a second peak top in a range of not less than 0.05 µm nor more than 1 µm.

### (Clause 3)

The cell according to clause 1 or clause 2, wherein
the porous membrane is an organic polymer porous membrane.

### (Clause 4)

The cell according to clause 3, wherein
when the cell is operated at a current density of 200 mA/cm² or more for 1000 hours or more, the operated cell has titanium in at least one pore of the porous membrane.

### (Clause 5)

The cell according to clause 4, wherein
an amount of the titanium in the at least one pore is defined by a mass ratio of a mass of any titanium compounds in the at least one pore to a mass of carbon in the organic polymer porous membrane, and the mass ratio is 0.0001 or more when the mass of carbon in the organic polymer porous membrane is assumed to 1.

### (Clause 6)

The cell according to clause 4, wherein:
the anode has a porous substrate; and
the porous substrate contains titanium and at least one element, the at least one element being selected from the group consisting of tantalum, vanadium, molybdenum, zirconium, nickel, niobium, ruthenium, palladium, platinum, gold, yttrium, and iron.

### (Clause 7)

The cell according to clause 5, wherein
when the porous membrane is divided in half thickness into a first porous part adjacent to the cathode and a second porous part adjacent to the anode, a mass of any titanium compounds in the second porous part is larger than a mass of any titanium compounds in the first porous part.

### (Clause 8)

The cell according to any one of clause 1 to clause 7, wherein
the cathode has:
   a porous substrate including carbon fibers;
   a diffusion layer disposed on the porous substrate; and
   a catalyst layer disposed on the diffusion layer,
the catalyst layer having a bulk density of 0.1 g/cm³ or more and less than 0.6 g/cm³.

### (Clause 9)

The cell according to clause 8, wherein
the porous substrate with the catalyst layer and the diffusion layer, has a bulk density of not less than 0.1 g/cm³ nor more than 0.7 g/cm³.

### (Clause 10)

The cell according to any one of clause 1 to clause 9, wherein
the first peak top is in a range of not less than 0.01 µm nor more than 0.2 µm, and the ISO air permeance is not less than 0.8 µm/Pa·s nor more than 100 µm/Pa·s.

### (Clause 11)

The cell according to clause 2, wherein
the second peak top is in a range of not less than 0.05 µm nor more than 0.8 µm.

### (Clause 12)

The cell according to any one of clause 1 to clause 11, wherein the reducible gas is carbon dioxide, and the substance to be oxidized is water or a hydroxide ion.

### (Clause 13)

The cell according to any one of clause 1 to clause 12, wherein
the ISO air permeability is not less than 1 µm/Pa·s nor more than 10 µm/Pa•s.

### (Clause 14)

The cell according to any one of clause 1 to clause 13, wherein
the first peak top is in a range of not less than 0.08 µm nor more than 0.25 µm.

### (Clause 15)

The cell according to clause 2, wherein
the second peak top is in a range of not less than 0.1 µm nor more than 0.25 µm.

### (Clause 16)

The cell according to any one of clause 1 to clause 15, wherein:
the cathode has a surface disposed on the separator; and
the anode has a surface disposed on the separator.

### (Clause 17)

The cell according to clause 3, wherein
the cell has a titanium oxide in at least one pore of the porous membrane.

### (Clause 18)

The cell according to any one of clause 1 to clause 17, wherein
the porous membrane includes a fluorocarbon resin, polyether, polysulfone, polyethylene, polypropylene, or cellulose.

### (Clause 19)

The cell according to clause 4, wherein
an amount of the titanium in the at least one pores is defined by a mass ratio of a mass of any titanium compounds in the at least one pore to a mass of carbon in the organic polymer porous membrane, the mass ratio being 0.0001 nor more than 0.001 when the mass of carbon in the organic polymer porous membrane is assumed to 1.

### (Clause 20)

An electrolysis device comprising:
the cell according to any one of clause 1 to clause19;
a gas supply configured to supply the reducible gas to a cathode flow path of the cell; and
an electrolytic solution supply configured to supply the electrolytic solution to an anode flow path of the cell.

## Claims

1. An electrolysis cell comprising:
a cathode configured to be in contact with a reducible gas and to reduce the reducible gas;
an anode configured to be in contact with an electrolytic solution containing an oxidizable substance and to oxidize the oxidizable substance, the anode containing titanium; and
a separator separating the cathode from the anode, wherein:
the separator includes a porous membrane;
the porous membrane gives a first pore size distribution defined by a first graph having a first horizontal axis and a first vertical axis, the first horizontal axis representing first pore sizes of through holes of the porous membrane, the first pore sizes being determined by the porometer, the first vertical axis representing a pore size flow distribution of pore volumes corresponding to the first pore sizes, and the first pore size distribution having a first peak top in not less than 0.01 µm nor more than 0.3 µm; and
the porous membrane has an ISO air permeance of not less than 0.8 µm/Pa·s nor more than 150 µm/Pa·s.

2. The cell according to claim 1, wherein
the porous membrane gives a second pore size distribution defined by a second graph having a second horizontal axis and a second vertical axis, the second horizontal axis representing second pore sizes of the porous membrane, the second pore sizes being determined by a mercury intrusion method, the second vertical axis representing log differential pore volumes corresponding to the second pore sizes, and the second pore size distribution having a second peak top in a range of not less than 0.05 µm nor more than 1 µm.

3. The cell according to claim 1 or claim 2, wherein
the porous membrane is an organic polymer porous membrane.

4. The cell according to claim 3, wherein
when the cell is operated at a current density of 200 mA/cm² or more for 1000 hours or more, the operated cell has titanium in at least one pore of the porous membrane.

5. The cell according to claim 4, wherein
an amount of the titanium in the at least one pore is defined by a mass ratio of a mass of any titanium compounds in the at least one pore to a mass of carbon in the organic polymer porous membrane, and the mass ratio is 0.0001 or more when the mass of carbon in the organic polymer porous membrane is assumed to 1.

6. The cell according to claim 4, wherein:
the anode has a porous substrate; and
the porous substrate contains titanium and at least one element, the at least one element being selected from the group consisting of tantalum, vanadium, molybdenum, zirconium, nickel, niobium, ruthenium, palladium, platinum, gold, yttrium, and iron.

7. The cell according to claim 5, wherein
when the porous membrane is divided in half thickness into a first porous part adjacent to the cathode and a second porous part adjacent to the anode, a mass of any titanium compounds in the second porous part is larger than a mass of any titanium compounds in the first porous part.

8. The cell according to any one of claim 1 to claim 7, wherein
the cathode has:
a porous substrate including carbon fibers;
a diffusion layer disposed on the porous substrate; and
a catalyst layer disposed on the diffusion layer,
the catalyst layer having a bulk density of 0.1 g/cm³ or more and less than 0.6 g/cm³.

9. The cell according to claim 8, wherein
the porous substrate with the catalyst layer and the diffusion layer, has a bulk density of not less than 0.1 g/cm³ nor more than 0.7 g/cm³.

10. The cell according to any one of claim 1 to claim 9, wherein
the first peak top is in a range of not less than 0.01 µm nor more than 0.2 µm, and the ISO air permeance is not less than 0.8 µm/Pa·s nor more than 100 µm/Pa•s.

11. The cell according to claim 2, wherein
the second peak top is in a range of not less than 0.05 µm nor more than 0.8 µm.

12. The cell according to any one of claim 1 to claim 11, wherein
the reducible gas includes carbon dioxide, and the oxidizable substance includes water or a hydroxide ion.

13. The cell according to any one of claim 1 to claim 12, wherein
the ISO air permeability is not less than 1 µm/Pa·s nor more than 10 µm/Pa•s.

14. The cell according to any one of claim 1 to claim 13, wherein
the first peak top is in a range of not less than 0.08 µm nor more than 0.25 µm.

15. An electrolysis device comprising:
the cell according to any one of claim 1 to claim 14;
a gas supply configured to supply the reducible gas to a cathode flow path of the cell; and
an electrolytic solution supply configured to supply the electrolytic solution to an anode flow path of the cell.
